

## UNITED STATES PATENT OFFICE

2,439,820

## COMPOUND LUBRICANTS

John M. Musselman, South Euclid, Ohio, assignor  
to The Standard Oil Company, Cleveland, Ohio,  
a corporation of Ohio

No Drawing. Application October 14, 1941,  
Serial No. 414,977

17 Claims. (Cl. 252—32.7)

1

In the preparation of metal compounds of the reaction product of a sulphide of phosphorus on a wax or sterol ester, I have found that the final products fall into two classes, in accordance with the particular metal, the properties and characteristics being of two different orders; and combinations of the two groups are of particular utility, providing combinations of properties not realized with compounds of one metal.

To the accomplishment of the foregoing and related ends, the invention, then, comprises the features hereinafter fully described, and particularly pointed out in the claims, the following description setting forth in detail certain illustrative embodiments of the invention, these being indicative however, of but a few of the various ways in which the principle of the invention may be employed.

The invention will be best understood by reference to an illustrative example: Phosphorus pentasulphide in amount of about 20 per cent is heated with neutral degras at approximately 300° F. for an hour. After separation of sludge, which is largely phosphorus pentoxide, the product, substantially free of phosphorus is reacted with about 5 per cent of arsenic trioxide and about 5 per cent of calcium oxide at a temperature of about 250° F. for an hour. After all constituents are combined, the product is clear. This product may be employed per se in extreme pressure gear usages etc., or it can be mixed with oils, combinations with heavy steam refined lubricating stock for instance giving particularly good results. In general, the amount of the metal compound may be 0.01 to 100 per cent in various usages.

The metals employed in the reaction may be applied in the form of oxides or other convenient reactive compounds, and as indicated above, there are two separate groups or categories. The compounds formed from metals below iron or copper in the E. M. F. series, as for example arsenic, antimony, bismuth, chromium, mercury, silver, etc., give products which are particularly protective against attack on metals to which the lubricant is applied, and they are also strikingly resistant against break-down of an oil with which they are incorporated. They may be regarded as antioxidants, using the term in a broad sense, without restricted implication that merely oxygen is the cause of break-down. The other metal com-

2

pounds, viz. those of metals not exceeding four electron orbits in groups I, II and III of the periodic system, as for instance calcium, sodium, potassium, aluminum, zinc, beryllium, magnesium, etc., as well as barium, give products which particularly have a detergent action or cleaning action on metal surfaces. Further illustrative advantageous combinations are antimony and aluminum, arsenic and barium, antimony and barium, chromium and calcium, chromium and barium, etc.

Instead of simultaneously reacting both metals with the reaction product of phosphorus sulphide and wax, the respective metals may be separately reacted with the reaction product of phosphorus sulphide and wax and the products may then be mixed. Equal portions may be employed, or depending upon the particular usages in view the proportions may be high for either the one type of metal compound or the other, as desired. The metal compounds may be applied without oil admixture, as in extreme pressure gear usages, or they may be mixed with oils, in desired amounts; and in general the amounts of the metal compounds may be 0.01 to 100 per cent, according to the usages.

As the wax raw material, aside from degras, other waxes, as lanolin, carnauba, Japan wax, sperm oil, etc., may be employed, the normally non-liquid waxes being particularly advantageous. The sulphide of phosphorus may be pentasulphide, sesquisulphide, etc., and as indicated the reaction is effected with heat, usually around 300° F., or somewhat higher or lower in some cases, and generally about an hour is required. The second reaction or conversion into the metal compounds also requires heat, as for instance 200 to 300° F., and usually for about an hour.

Other modes of applying the principle of the invention may be employed, change being made as regards the details described, provided the features stated in any of the following claims or the equivalent of such, be employed.

I therefore particularly point out and distinctly claim as my invention:

1. Compounds of a heavy metal selected from the group consisting of chromium and metals below iron in the E. M. F. series and of a metal selected from the group consisting of barium and metals having not more than four electron orbits

selected from groups I, II and III of the periodic system, and the reaction product of a sulphide of phosphorus and an oxygen-containing wax reacted at a temperature to separate a phosphorus and oxygen-containing residue.

2. A lubricant comprising a lubricating oil containing an additive in an amount to improve the stability of the oil under conditions of usage, said additive comprising compounds of a heavy metal selected from the group consisting of chromium and metals below iron in the E. M. F. series and of a metal selected from the group consisting of barium and metals having not more than four electron orbits selected from groups I, II and III of the periodic system, and the reaction product of phosphorus pentasulphide and an oxygen-containing wax reacted at a temperature to separate a phosphorus and oxygen-containing residue.

3. Compounds of arsenic and of calcium and the reaction product of a sulphide of phosphorus and an oxygen-containing wax reacted at a temperature to separate a phosphorus and oxygen-containing residue.

4. Compounds of antimony and of barium, and the reaction product of a sulphide of phosphorus and an oxygen-containing wax reacted at a temperature to separate a phosphorus and oxygen-containing residue.

5. Compounds of chromium and of barium, and the reaction product of a sulphide of phosphorus and an oxygen-containing wax reacted at a temperature to separate a phosphorus and oxygen-containing residue.

6. Compounds of a heavy metal selected from the group consisting of chromium and metals below iron in the E. M. F. series and of a metal selected from the group consisting of barium and metals having not more than four electron orbits selected from groups I, II and III of the periodic system, and the reaction product of a sulphide of phosphorus and degras reacted at a temperature to separate a phosphorus and oxygen-containing residue.

7. A lubricant comprising a lubricating oil containing an additive in an amount to improve the stability of the oil under conditions of usage, said additive comprising compounds of a heavy metal selected from the group consisting of chromium and metals below iron in the E. M. F. series and of a metal selected from the group consisting of barium and metals having not more than four electron orbits selected from groups I, II and III of the periodic system, and the reaction product of phosphorus pentasulphide and degras reacted at a temperature to separate a phosphorus and oxygen-containing residue.

8. Compounds of arsenic and of calcium, and the reaction product of a sulphide of phosphorus and degras reacted at a temperature to separate a phosphorus and oxygen-containing residue.

9. Compounds of antimony and of barium, and the reaction product of a sulphide of phosphorus and degras reacted at a temperature to separate a phosphorus and oxygen-containing residue.

10. Compounds of chromium and of barium, and the reaction product of a sulphide of phosphorus and degras reacted at a temperature to separate a phosphorus and oxygen-containing residue.

11. Compounds of a heavy metal selected from the group consisting of chromium and metals below iron in the E. M. F. series and of a metal having not more than four electron orbits selected from groups I, II and III of the periodic system,

and the reaction product of a sulphide of phosphorus and an oxygen-containing wax.

12. The process for making a composition of matter suitable for use as a lubricant or as an addition agent to improve the characteristics of lubricating oil, comprising reacting a sulphide of phosphorus with an oxygen-containing wax at a temperature to convert the phosphorus to a phosphorus and oxygen-containing compound which separates in a residue removing said residue from the reaction product, and reacting said product with compounds of a heavy metal selected from the group consisting of chromium and metals below iron in the E. M. F. series and of a metal having not more than six electron orbits selected from groups I, II and III of the periodic system, to form the corresponding metal compounds of said first reaction product.

13. The process for making a composition of matter suitable for use as a lubricant or as an addition agent to improve the characteristics of lubricating oil, comprising reacting phosphorus pentasulphide with an oxygen-containing wax at a temperature to convert the phosphorus to an oxide, removing said residue from the reaction product, and reacting said product with compounds of a heavy metal selected from the group consisting of chromium and metals below iron in the E. M. F. series and of a metal having not more than six electron orbits selected from groups I, II and III of the periodic system, to form the corresponding metal compounds of said first reaction product.

14. The process for making a composition of matter suitable for use as a lubricant or as an addition agent to improve the characteristics of lubricating oil, comprising reacting a sulphide of phosphorus with degras at a temperature to convert the phosphorus to a phosphorus and oxygen-containing compound which separates in a residue removing said residue from the reaction product, and reacting said product with compounds of a heavy metal selected from the group consisting of chromium and metals below iron in the E. M. F. series and of a metal having not more than six electron orbits selected from groups I, II and III of the periodic system, to form the corresponding metal compounds of said first reaction product.

15. The process for making a composition of matter suitable for use as a lubricant or as an addition agent to improve the characteristics of lubricating oil, comprising reacting a sulphide of phosphorus with degras at a temperature to convert the phosphorus to a phosphorus and oxygen-containing compound which separates in a residue removing said residue from the reaction product, and reacting said product with compounds of arsenic and of calcium to form arsenic and calcium compounds of said first reaction product.

16. The process for making a composition of matter suitable for use as a lubricant or as an addition agent to improve the characteristics of lubricating oil, comprising reacting a sulphide of phosphorus with degras at a temperature to convert the phosphorus to a phosphorus and oxygen-containing compound which separates in a residue removing said residue from the reaction product, and reacting said product with compounds of antimony and of barium to form antimony and barium compounds of said first reaction product.

17. The process for making a composition of matter suitable for use as a lubricant or as an

addition agent to improve the characteristics of lubricating oil, comprising reacting a sulphide of phosphorus with degras at a temperature to convert the phosphorus to a phosphorus and oxygen-containing compound which separates in a residue removing said residue from the reaction product, and reacting said product with compounds of chromium and of barium to form chromium and barium compounds of said first reaction product.

JOHN M. MUSSELMAN.

UNITED STATES PATENTS

|   | Number    | Name      | Date          |
|---|-----------|-----------|---------------|
| 5 | 2,237,096 | Dearborn  | Apr. 1, 1941  |
|   | 2,331,923 | Musselman | Oct. 19, 1943 |
|   | 2,263,445 | Reiff     | Nov. 18, 1941 |
|   | 2,257,751 | Lincoln   | Oct. 7, 1941  |
|   | 2,211,306 | Whittier  | Aug. 13, 1940 |
|   | 1,767,076 | Jarman    | June 24, 1930 |

10

FOREIGN PATENTS

| Number  | Country       | Date         |
|---------|---------------|--------------|
| 521,656 | Great Britain | May 28, 1940 |

OTHER REFERENCES

The following references are of record in the file of this patent:

16      Handbook of Chemistry and Physics, Hodgman, 21st ed., page 695.

REFERENCES CITED

Certificate of Correction

Patent No. 2,439,820.

April 20, 1948.

JOHN M. MUSSELMAN

It is hereby certified that error appears in the printed specification of the above numbered patent requiring correction as follows: Column 3, line 73, claim 11, after the word "metal" insert *selected from the group consisting of barium and metals*; and that the said Letters Patent should be read with this correction therein that the same may conform to the record of the case in the Patent Office.

Signed and sealed this 15th day of June, A. D. 1948.

[SEAL]

THOMAS F. MURPHY,  
*Assistant Commissioner of Patents.*

addition agent to improve the characteristics of lubricating oil, comprising reacting a sulphide of phosphorus with degras at a temperature to convert the phosphorus to a phosphorus and oxygen-containing compound which separates in a residue removing said residue from the reaction product, and reacting said product with compounds of chromium and of barium to form chromium and barium compounds of said first reaction product.

JOHN M. MUSSELMAN.

UNITED STATES PATENTS

|   | Number    | Name      | Date          |
|---|-----------|-----------|---------------|
| 5 | 2,237,096 | Dearborn  | Apr. 1, 1941  |
|   | 2,331,923 | Musselman | Oct. 19, 1943 |
|   | 2,263,445 | Reiff     | Nov. 18, 1941 |
|   | 2,257,751 | Lincoln   | Oct. 7, 1941  |
|   | 2,211,306 | Whittier  | Aug. 13, 1940 |
|   | 1,767,076 | Jarman    | June 24, 1930 |

10

FOREIGN PATENTS

| Number  | Country       | Date         |
|---------|---------------|--------------|
| 521,656 | Great Britain | May 28, 1940 |

OTHER REFERENCES

The following references are of record in the file of this patent:

16      Handbook of Chemistry and Physics, Hodgman, 21st ed., page 695.

REFERENCES CITED

Certificate of Correction

Patent No. 2,439,820.

April 20, 1948.

JOHN M. MUSSELMAN

It is hereby certified that error appears in the printed specification of the above numbered patent requiring correction as follows: Column 3, line 73, claim 11, after the word "metal" insert *selected from the group consisting of barium and metals*; and that the said Letters Patent should be read with this correction therein that the same may conform to the record of the case in the Patent Office.

Signed and sealed this 15th day of June, A. D. 1948.

[SEAL]

THOMAS F. MURPHY,  
*Assistant Commissioner of Patents.*